

# United States Patent

[11] 3,619,279

[72] Inventors **Herbert N. Johnston**  
Columbus;  
**Nicholas D. Gallagher, Troy, both of Ohio**  
842,356

[21] Appl. No. 842,356

[22] Filed July 16, 1969

Division of Ser. No. 520,872 Jan. 17, 1966, Pat. No. 3,493,412

[45] Patented Nov. 9, 1971

[73] Assignee **Xerox Corporation**  
Rochester, N.Y.

[54] **TONER RECEIVING MEMBER**  
10 Claims, No Drawings

[52] U.S. Cl. .... 117/155 UA,  
117/154, 117/156

[51] Int. Cl. .... D21h 1/34,  
G03g 7/00

[50] Field of Search.... 117/33, 76  
P, 155 U, 156, 154

[56]

## References Cited

### UNITED STATES PATENTS

|           |         |                      |           |
|-----------|---------|----------------------|-----------|
| 1,783,442 | 12/1930 | Mayer et al.....     | 117/167 X |
| 2,462,029 | 2/1949  | Perry.....           | 117/155 X |
| 2,833,671 | 5/1958  | Funk et al.....      | 117/79 X  |
| 2,875,168 | 2/1959  | Smith et al.....     | 260/31.4  |
| 2,885,306 | 5/1959  | Rigterink et al..... | 117/122   |
| 2,914,436 | 11/1959 | Nakiclny .....       | 117/144 X |
| 3,130,064 | 4/1964  | Insalaco .....       | 117/17.5  |
| 3,260,612 | 7/1966  | Dulmage et al.....   | 117/33 X  |
| 3,336,152 | 8/1967  | Garden.....          | 117/121 X |

Primary Examiner—William D. Martin

Assistant Examiner—M. R. Lusighan

Attorneys—James J. Ralabate, Albert A. Mahassel and Samuel E. Mott

**ABSTRACT:** A toner receiving member having available at an external surface a solid crystalline plasticizer to reduce the fusion power requirements when toner is fused to the receiving member. The external surface of the toner receiving member is substantially free of material plasticizable by the solid crystalline plasticizer. Typically a plasticizer such as ethylene glycol dibenzoate may be available on the surface of paper.

## TONER RECEIVING MEMBER

This application is a division of copending application Ser. No. 520,872, filed Jan. 17, 1966, now U.S. Pat. No. 3,493,412.

This invention relates in general to imaging systems, and more particularly, to improved receiving surfaces, their manufacture and use.

The formation and development of images on the surface of photoconductive materials by electrostatic means is well known. The basic xerographic process as taught by C. F. Carlson in U.S. Pat. No. 2,297,691 involves placing a uniform electrostatic charge on a photoconductive insulating layer, exposing the layer to a light and shadow image to dissipate the charge on the areas of the layer exposed to the light and developing the resulting latent electrostatic image by depositing on the image a finely divided electroscopic material referred to in the art as "toner." The toner will normally be attracted to those areas of the layer which retain a charge, thereby forming a toner image corresponding to the latent electrostatic image. This powder may then be transferred to a receiving surface such as paper. The transferred image may subsequently be permanently affixed to the support surface as by heat. Instead of latent image formation by uniformly charging the photoconductive layer and then exposing the layer to a light and shadow image, one may form the latent image by directly charging the layer in image configuration. Several methods are known for applying the electroscopic particles to the latent electrostatic image to be developed. These methods include "cascade" development, "magnetic brush" development, "powder cloud" development and "liquid" development as described in U.S. Pat. Nos. 2,618,552; 2,874,063; 2,221,776; and 2,891,911 respectively. The processes mentioned above together with numerous variations are well known to the art through various patents and publications and through the widespread availability and utilization of electrostatic imaging equipment.

A variety of types of finely divided electroscopic powders are disclosed in the Carlson patent. However, as the art of electrostatic copying has progressed, a variety of pigmented thermoplastic resins have evolved as the preferred toner materials when heat is employed to fuse the thermoplastic toner image to a support surface. While ordinarily capable of producing excellent quality images, these toner materials possess serious deficiencies in certain areas. When the toner is to be fused onto an inflammable surface such as paper, the toner resin should have a fusing temperature below the thermal degradation temperature of the paper. Upon heating to the discoloration temperature or flame point of some papers, resinous toners having high fusing temperatures often do not become sufficiently fluid to penetrate and adhere to the paper. The resulting powdery and incompletely fused images are easily removed by rubbing. On the other hand, toner resins having low fusing temperatures are usually tacky at ordinarily encountered ambient temperatures and form undesirable agglomerates during storage and handling. Additionally, images on copies manufactured from tacky toners have a tendency to offset onto adjacent surfaces. Some tacky toners form smears on reusable electrophotographic imaging surfaces which are difficult to remove. Where the toner materials smears excessively, a film of toner material builds up on the electrophotographic surface. This film has different electrical characteristics than the plate and, if hydroscopic in nature, detrimentally affects the conductivity of the electrophotographic surface when relative humidity is high. Thermoplastic resins having consistently uniform molecular weights are difficult to manufacture. Since thermoplastic resins are usually an amorphous mixture of polymer chains having different molecular weights and normally possess a nonuniform melting range rather than a sharp melting point, it is difficult to accurately predict the temperature at which any given polymeric thermoplastic resin will fuse and adhere to a receiving sheet. Toners having erratic fusing temperatures and wide fusing temperature ranges require that the machines have a built-in fusing safety factor. Since the temperature in the fuser cannot

be raised above the char point of the paper, this often imposes an undesirably low upper limit on the speed of the paper through the fuser. Further, the heat fusing units currently employed to fuse conventional thermoplastic toners often cause

- 5 the temperature of poorly ventilated rooms to reach levels which shorten machine component life and contribute to operator discomfort. It is known, as disclosed in U.S. Pat. No. 3,130,064 to improve toner fusing at lower temperatures by employing business machine record cards treated with thermoplastic resins dissolved in organic solvents. Unlike a plasticizer, the thermoplastic resin apparently functions as a melting agent with "like melting like." Although the disclosed plastic resin films may reduce toner fixing temperatures, the thermoplastic resin melting range problems described above have not been obviated. Pencil and ink markings are difficult 10 to apply and remove from surfaces coated with the thermoplastic resin films. Also, more complex equipment and specially designed paper making processes are required when the thermoplastic resin films are applied with inflammable, expensive and toxic organic solvents. Since most thermoplastic toner particles, receiving sheets, and developing processes are deficient in one or more of the above areas, there is a continuing 15 need for a better system for fusing toner images.

20 It is, therefore, an object of this invention to provide a receiving surface overcoming the above-noted deficiencies.

It is another object of this invention to provide a receiving surface which reduces the quantity of heat energy necessary to fuse toner images.

25 It is another object of this invention to provide a receiving surface which effectuates uniform and sharp toner fusion temperatures.

It is another object of this invention to provide a receiving surface which is receptive to ink and pencil markings.

30 It is another object of this invention to provide a receiving surface which is easily erasable.

It is another object of this invention to provide a receiving surface which allows the employment of cooler, more compact toner fusing units.

35 It is another object of this invention to provide a receiving surface which permits the use of higher electrophotographic imaging machine speeds.

It is another object of this invention to provide a receiving surface which allows the employment of high melting non-tacky toners.

40 It is another object of this invention to provide a receiving surface having physical and chemical properties superior to those of known receiving sheets.

45 The above objects and others are accomplished, generally speaking, by providing a receiving surface treated with a solid crystalline plasticizer which effectuates complete thermoplastic toner fusion under heating conditions at which untreated surfaces afford only marginal or no fusion. Crystalline plasticizers, which separate from the thermoplastic resins

50 when the plasticized resin is cooled to room temperature are used because tacky images and attendant offset problems are then avoided. It is believed that separation occurs in the form of tiny islands of crystalline plasticizer particles in a matrix of toner material. Although it is not clear, it is believed that when solid, crystalline plasticizers are heated above their melting point, they weaken the Van der Waal forces existing in the thermoplastic toner polymers and allow slippage of the long linear polymer chains thereby promoting fluidity at lower temperatures.

55 Experiments have revealed that some liquid plasticizers provide virtually complete toner fusion under heating conditions at which untreated receiving surfaces give only marginal fusion, but the resulting image is either permanently tacky or tacky for extended periods of time. Receiving surfaces carrying tacky images plasticized with liquid plasticizers will offset toner material to adjacent surfaces and cause feathering of the images. Additionally, the nonimaged areas of receiving surfaces treated with liquid plasticizer will at room temperature actively soften and render tacky any thermoplastic image on adjacent surfaces. A solid crystalline

plasticizer having a melting point greater than about 45° C. is preferred, because premature melting and activation during storage is avoided and rapid plasticizer recrystallization in toner images is promoted. To be effective, the solid plasticizer should have a melting point below the melting range of the thermoplastic toner resin. The uniform and sharp melting point characteristics of crystalline plasticizers permit the employment of cooler and more efficient fusing units in precision electrostatic imaging machines.

Outstanding results have been obtained with ethylene glycol dibenzoate (EGDB) and blends of EGDB and diphenyl phthalate (DPP). When receiving surfaces treated with EGDB are employed, the speed of existing electrophotographic copying machines have been more than doubled. Additionally, EGDB recrystallizes in seconds when cooled to room temperature. Other suitable solid plasticizers may, however, be substituted for EGDB. Typical solid, crystalline plasticizers include: ethylene glycol dibenzoate, dimethyl isophthalate (DMIP), glycerol tribenzoate, dicyclohexyl phthalate (DCHP), diphenyl phthalate, and blends thereof.

Any suitable receiving surface may be treated with the plasticizer material of this invention. For example, the surface of sheets, webs, planks, or even massive objects may be coated or impregnated with the solid plasticizer of this invention. The receiving surface may be composed of any suitable organic material, inorganic material, or mixtures thereof. If the receiving surface contains a thermoplastic resin, it may be desirable to select a plasticizer which does not plasticize and distort the receiving surface. Conversely, distortion of the receiving surface may be deliberately induced to achieve a desired decorative effect.

The plasticizer composition may be applied to the receiving surface by any conventional method such as spraying, electrostatic deposition, dipping, fluidized bed coating, brushing, or roll coating. Further, the plasticizer may be added to the receiving surface in any suitable manner prior to, during, or subsequent to the manufacture of the receiving surface. For example, the plasticizer may be applied alone or in combination with other materials as a powder, dispersion, solution, vapor, emulsion, or melt to paper during or after the papermaking process. Optimum results have been obtained when the plasticizer is applied admixed with a binder because the problem of dust contamination is eliminated. Any suitable binder may be employed to immovably attach the solid plasticizer to the receiving surface. Typical binders include: acetylated starch, styrene-butadiene latex, carboxy-methyl cellulose, polyvinyl pyrrolidone, acrylic latex, polyvinyl acetate copolymers, polyvinyl alcohol, soy proteins, casein, hydroxyethylated starch and mixtures thereof. Any of the conventional additives such as antioxidants, emulsifiers,

brighteners, solvents, surfactants, suspending agents, antifoam agents, coloring agents and fillers may be employed with the binder. Binders comprising acetylated starch, styrene-butadiene copolymers, polyvinyl pyrrolidone, casein, polyvinyl alcohol and mixtures thereof are preferred because they are very stable in conventional high-speed paper coating apparatus. Surprisingly, toner images formed on receiving surfaces treated with a binder and plasticizer mixtures are more dense than toner images formed on untreated receiving surfaces. Additionally, paper sheets treated with a binder and plasticizer mixture lie flatter after toner fusion than untreated paper. It is preferred that the binder content remain below about 40 percent, based on the weight of the plasticizer, as this provides much more efficient fusing apparently because plasticizer is available at the surface where the toner is to be fused to the receiving member.

Paper sheets or webs are normally employed as the receiving surface in most conventional electrostatic imaging processes. The paper may comprise organic and/or inorganic fibers such as cellulose, modified cellulose, polymeric resin, glass, and asbestos fibers. The plasticizer may be added to paper at any stage of the papermaking process. Surface coatings containing at least about 0.4 pound of plasticizer per ream (500 17 in.×22 in. sheets, 1,300 square feet) will markedly reduce toner fusion power requirements although smaller amounts may also have some effect. When the plasticizer material is incorporated into the paper prior to sheet formation, e.g., in the beater, or subsequent to web formation, e.g., by impregnation, proportionately more plasticizer is necessary in order to maintain a sufficient quantity of plasticizer at the surface of the paper sheet. Excellent results are obtained when from about 0.5 to about 1.5 pounds of plasticizer per 1,300 square feet is applied to receiving surfaces as a surface coating.

Electroscopic toner compositions are well known to those skilled in the art. among the patents describing such compositions are U.S. Pat. No. 2,618,551 to Walkup, U.S. Pat. No. 2,618,552 to Wise, U.S. Pat. No. 2,638,415 to Walkup and Wise, U.S. Pat. No. 2,659,670 to Copley, and U.S. Pat. No. 2,788,415 to Rheinfrank and Jones. These toners generally have an average particle diameter between 1 and 30 microns. Clearly, the plasticizer treated receiving surface should be used with those thermoplastic resin toners which will be plasticized by the specific plasticizer employed in the receiving surface. Selection of compatible combinations of solid crystalline plasticizer and thermoplastic resin toner will be obvious to those skilled in the art. Blends of two or more plasticizers may be used to broaden the toner spectrum of the receiving surface. Typical thermoplastic resins include: acrylic resins, methacrylic resins, cellulose acetate, cellulose nitrate,

#### TONER FUSION EFFECTS OBTAINED ON PAPER TREATED WITH PLASTICIZERS

| Examples | Grind*                | Plasticizer compositions, parts by weight |                                          |                   | Power index, watts/(in./sec.) | Toner fusion results                     |
|----------|-----------------------|-------------------------------------------|------------------------------------------|-------------------|-------------------------------|------------------------------------------|
|          |                       | Styrene-butadiene latex (Dow 636)         | Polyvinyl pyrrolidone, 20% solids (K-30) | Acetylated starch |                               |                                          |
| I        |                       |                                           |                                          |                   | 500                           | Fuses, no rub off, non-tacky.            |
| II       |                       |                                           |                                          |                   | 250                           | Very poor fusing, powdery rub off.       |
| III      | 80 (DPP)              |                                           |                                          | 20                | 133                           | Good fusing, no rub off, slightly tacky. |
| IV       | 80 (DCHP)             |                                           |                                          | 4.2               | 133                           | Do.                                      |
| V        | 80 (EGDB)             |                                           |                                          | 6.5               | 125                           | Good fusing, no rub off, non-tacky.      |
| VI       | 7 (DPP) and 73 (EGDB) |                                           |                                          | 6.5               | 115                           | Do.                                      |
| VII      | 299 (DMIP)            |                                           |                                          | 51                | 276                           | Do.                                      |
| VIII     | 80 (EGDB)             |                                           |                                          | 15                | 130                           | Do.                                      |
| IX       | 80 (EGDB)             |                                           |                                          | 30                | 225                           | Do.                                      |

\*Prepared by diluting ball mill grinds of the following compositions (parts by weight) with the indicated additives:

| Plasticizer                                  | Dicyclohexyl phthalate (DCHP) grind | Diphenyl phthalate (DPP) grind | Ethylene glycol dibenzoate (EGDB) grind | Dimethyl isophthalate (DMIP) grind |
|----------------------------------------------|-------------------------------------|--------------------------------|-----------------------------------------|------------------------------------|
| Sodium salt of processed rosin (Dresinate X) | 150                                 | 150                            | 150                                     | 150                                |
| Polyvinyl pyrrolidone (PVP type K-130)       | 1                                   | 1                              | 1                                       | 1                                  |
| Water                                        | 2                                   | 2                              | 2                                       | 2                                  |
|                                              | 147                                 | 147                            | 277                                     | 146                                |

polystyrene, polyethylene, polypropylene, polycarbonate, modified phenolformaldehyde resins and mixtures thereof.

The following examples further define, describe and compare exemplary methods of preparing the receiving surfaces of the present invention and of utilizing them as substrates for electrostatic latent images. Parts and percentages are by weight unless otherwise indicated.

In the following, examples I-IX are carried out with a toner comprising a styrene and n-butylmethacrylate copolymer, polyvinyl butyral, and carbon black prepared by the method disclosed by M. A. Insalaco in example I of U.S. Pat. No. 3,079,342. The treated receiving sheets carry a surface coating of a plasticizer mixture applied as an aqueous dispersion by means of a smooth metal reverse roll in a Dietzco-Dixon Pilot Coated followed by doctoring with a reverse rotating No. 4 wire-wound and finally dried by heated air. The electrostati-

In the following examples X-XXXIX, sheets treated with the compositions in table A are compared with untreated sheets. Different quantities of treatment material per ream and various transport speeds are employed to demonstrate how these two factors affect fusing energy requirements. The power index required to obtain equivalent fusion with untreated paper is determined by comparing the rub off from a treated sheet with a standardized rub off series obtained with untreated sheets. The images on untreated and treated sheets are deemed equivalent when the quantity of rub off from each is identical. The toner material is rubbed off by drawing a 2-inch square cloth (Crockmeter Square, Test Fabrics, Inc.) weighted with a 500 gram balance weight across and along an 11-inch length of the images sheet. The percentage reduction in power input required to obtain equivalent fusion was calculated according to the following formula:

Percent reduction in power =

Power index required to obtain equivalent fusion with untreated paper minus power index used

Power index required to obtain equivalent fusion with untreated paper

TABLE A.—PLASTICIZER COMPOSITIONS  
[Parts by weight]

| Treatment system | Ethylene dibenzoate | Polyvinyl pyrrolidone, (K-30) | Sodium salt of processed resin (Dresinate X) | Hydroxyethyl derivative of corn starch (Penford Gum 280) | Polyvinyl alcohol, Elvanol 72-60 | Styrene-butadiene latex (Dow 636) |
|------------------|---------------------|-------------------------------|----------------------------------------------|----------------------------------------------------------|----------------------------------|-----------------------------------|
| (1)              | 840.0               | 11.2                          | 5.6                                          | -----                                                    | -----                            | 2,051.2                           |
| (2)              | 840.0               | 11.2                          | 5.6                                          | -----                                                    | -----                            | 1,551.2                           |
| (3)              | 840.0               | 11.2                          | 5.6                                          | -----                                                    | -----                            | 2,051.2                           |
| (4)              | 840.0               | 11.2                          | 5.6                                          | 31.7                                                     | -----                            | 2,051.2                           |
| (5)              | 840.0               | 11.2                          | 5.6                                          | -----                                                    | 31.7                             | 2,051.2                           |

TONER FUSION PROPERTIES OBTAINED WITH PAPERS TREATED WITH PLASTICIZERS

| Examples | Treatment system applied* | Treatment level, lbs./ream | Power settings used | Power watts, port speed, in./sec. | Trans- | Corre- | Power index required to obtain equivalent fusion with untreated paper | Reduction in power input, percent |
|----------|---------------------------|----------------------------|---------------------|-----------------------------------|--------|--------|-----------------------------------------------------------------------|-----------------------------------|
| X        | -----                     | -----                      | -----               | 864                               | 1.7    | 508    | 508                                                                   | 0                                 |
| XI       | -----                     | -----                      | -----               | 864                               | 1.4    | 617    | 617                                                                   | 0                                 |
| XII      | -----                     | -----                      | -----               | 864                               | 1.1    | 783    | 783                                                                   | 0                                 |
| XIII     | -----                     | -----                      | -----               | 864                               | 1.7    | 508    | 718                                                                   | 29.0                              |
| XIV      | (2)                       | 1.99                       | -----               | 864                               | 1.4    | 617    | 718                                                                   | 14.1                              |
| XV       | (2)                       | -----                      | -----               | 864                               | 1.1    | 783    | 718                                                                   | 45.6                              |
| XVI      | (1)                       | 0.84                       | -----               | 864                               | 1.7    | 508    | 718                                                                   | 29.0                              |
| XVII     | (1)                       | -----                      | -----               | 864                               | 1.4    | 617    | 957                                                                   | 35.6                              |
| XVIII    | (1)                       | -----                      | -----               | 864                               | 1.1    | 783    | 957                                                                   | 18.2                              |
| XIX      | (1)                       | 0.94                       | -----               | 864                               | 1.7    | 508    | 664                                                                   | 21.3                              |
| XX       | (1)                       | -----                      | -----               | 864                               | 1.4    | 617    | 718                                                                   | 14.1                              |
| XXI      | (1)                       | -----                      | -----               | 864                               | 1.1    | 783    | 1,149                                                                 | 31.9                              |
| XXII     | (3)                       | 1.15                       | -----               | 864                               | 1.7    | 508    | 718                                                                   | 29.8                              |
| XXIII    | (3)                       | -----                      | -----               | 864                               | 1.4    | 617    | 862                                                                   | 28.5                              |
| XXIV     | (3)                       | -----                      | -----               | 864                               | 1.1    | 783    | 718                                                                   | 45.6                              |
| XXV      | (3)                       | 0.54                       | -----               | 864                               | 1.7    | 508    | 640                                                                   | 20.1                              |
| XXVI     | (3)                       | -----                      | -----               | 864                               | 1.4    | 617    | 957                                                                   | 35.6                              |
| XXVII    | (3)                       | -----                      | -----               | 864                               | 1.1    | 783    | 1,149                                                                 | 31.9                              |
| XXVIII   | (3)                       | 0.69                       | -----               | 864                               | 1.7    | 508    | 783                                                                   | 35.2                              |
| XXIX     | (3)                       | -----                      | -----               | 864                               | 1.4    | 617    | 957                                                                   | 35.6                              |
| XXX      | (3)                       | -----                      | -----               | 864                               | 1.1    | 783    | 1,149                                                                 | 31.9                              |
| XXXI     | (3)                       | 0.89                       | -----               | 864                               | 1.7    | 508    | 862                                                                   | 41.1                              |
| XXXII    | (3)                       | -----                      | -----               | 864                               | 1.4    | 617    | 862                                                                   | 28.5                              |
| XXXIII   | (3)                       | -----                      | -----               | 864                               | 1.1    | 783    | 718                                                                   | 45.6                              |
| XXXIV    | (4)                       | 0.84                       | -----               | 864                               | 1.7    | 508    | 783                                                                   | 35.2                              |
| XXXV     | (4)                       | -----                      | -----               | 864                               | 1.4    | 761    | 957                                                                   | 35.6                              |
| XXXVI    | (4)                       | -----                      | -----               | 864                               | 1.1    | 783    | >1,438                                                                | >45.6                             |
| XXXVII   | (5)                       | -----                      | -----               | 864                               | 1.7    | 508    | 862                                                                   | 41.1                              |
| XXXVIII  | (5)                       | -----                      | -----               | 864                               | 1.4    | 617    | 957                                                                   | 35.6                              |
| XXXIX    | (5)                       | -----                      | -----               | 864                               | 1.1    | 783    | >1,438                                                                | >45.6                             |

\* See Table A.

cally imaged sheets are passed at selected speeds under a quartz filament infrared heater unit operated with a fixed power input. For comparative evaluations, a "power index" value is assigned to the fusing conditions employed. The power index value is computed as follows:

$$\text{Power index, watts/(in./sec.)} = \frac{\text{Power input (watts)}}{\text{Transport speed (in./sec.)}}$$

Tack and the quantity of powder rub off of the fused images onto cotton are also compared.

#### EXAMPLE XXX

Paper sheets are treated with ethyl phthalyl ethyl glycolate, a liquid plasticizer, by dipping the sheets into a methyl alcohol solution containing about 10 percent by weight of the plasticizer. After the alcohol solvent is driven off, an electrostatically deposited styrene copolymer toner image is transferred to the treated sheet. The sheet is then heated on the back side with a bar type heater for 5 seconds at 125° C. The toner image is completely fused under these heating condi-

tions. With untreated paper, the same heating conditions provide only marginal fusion of the toner image. However, upon aging, the paper treated with the liquid plasticizer is found to offset toner to adjacent sheets and cause feathering of ink images.

#### EXAMPLE XXXI

Paper sheets are treated with cresyl diphenyl phosphate, a liquid plasticizer, by dipping the sheets into a methyl alcohol solution containing about 9 percent by weight of the plasticizer. After the alcohol solvent is driven off, an electrostatically deposited styrene copolymer toner image is transferred to the treated sheet. The sheet is then heated on a back side with a bar type heater for 5 seconds at 125° C. The toner image is completely fused under these heating conditions. With untreated paper under these same heating conditions, only marginal fusion of the toner image is obtained. However, upon aging, the paper treated with the liquid plasticizer is found to offset toner to adjacent sheets and cause feathering of ink images.

#### EXAMPLE XXXII

Paper treated with a plasticizer composition containing about 1,080 parts EGDB, 14.4 parts polyvinyl pyrrolidone (K-30), 340 parts butadiene-styrene latex, 0.14 part brightner (Calcofluor White CBP), 5 parts ammonium hydroxide (28 percent), 7.2 parts polymerized sodium salt of an alkyl naphthalene sulfonic acid (Daxad 11) and 1,083 parts water is imaged with a styrene copolymer toner in a Xerox 813 electrophotographic copier machine (similar to the machine described in U.S. Pat. No. 3,099,943) at a 12 copies per minute speed. This speed is twice the normal speed of the Xerox 813 copier. The toner image is fused and nontacky. No toner fix whatever is obtained with standard office bond paper run in the same machine at the same speed.

#### EXAMPLE XXXIII

A rosin-modified phenol-formaldehyde resin toner prepared in the manner disclosed in example I of U.S. Pat. No. 2,753,308 is imaged onto a paper sheet treated with the EGDB composition of example V above. Upon heating between two parallel heating plates, spaced 1 inch apart, the toner fuses more rapidly on the treated paper than on untreated paper under substantially identical heating conditions.

#### EXAMPLE XXXIV

A styrene-methyl methacrylate copolymer toner is imaged onto a paper sheet treated with the EGDB composition of example VIII above. Upon heating between two parallel heater plates, spaced 1 inch apart, the toner fuses more rapidly on the treated paper than on untreated paper under substantially identical heating conditions.

Although specific materials and conditions are set forth in the foregoing examples, these are merely intended as illustrations of the present invention. Various other suitable ther-

moplastic resin toners, receiving surfaces, plasticizers, binders, and coating processes such as those listed above may be substituted for those in the examples with similar results. Other materials may also be added to the base, plasticizer, binder or toner to sensitize, synergize or otherwise improve the fusing properties or other desirable properties of the system.

Other modifications of the present invention will occur to those skilled in the art upon a reading of the present disclosure. These are intended to be included within the scope of this invention.

We claim:

1. A toner image receiving member capable of producing nontacky images with no rub off comprising a paper base and adhered thereto and available at an external surface of said base at least one solid crystalline plasticizer, said solid crystalline plasticizer being a plasticizer for finely divided thermoplastic toner particles when said plasticizer and said toner particles are fused together, said plasticizer having a melting point of at least about 45° C. and below the melting range of said thermoplastic resin toner and being present in an amount of at least about 0.4 pound per 1,300 square feet of said external surface of said base, said solid crystalline plasticizer being capable of rapidly recrystallizing after being cooled below the melting point, said external surface of said base being free of material plasticizable by said solid crystalline plasticizer.
2. A toner image receiving member according to claim 1 wherein said solid crystalline plasticizer is adhered to at least the surface of said member by means of a binder composition, said binder composition being free of material plasticizable by said solid crystalline plasticizer.
3. A toner image receiving member according to claim 2 wherein said solid crystalline plasticizer is adhered to said toner receiving member by less than about 40 percent by weight of said binder, based on the weight of said plasticizer.
4. A toner image receiving member according to claim 1 wherein said solid crystalline plasticizer is available at said image receiving member as a powder.
5. A toner image receiving member according to claim 1 wherein said base comprises a paper web.
6. A toner image receiving member according to claim 2 wherein said binder composition comprises a binder selected from the group consisting of polyvinyl pyrrolidone, styrene butadiene copolymer, acetylated starch, casein, polyvinyl alcohol, and mixtures thereof.
7. A toner image receiving member according to claim 1 wherein said solid crystalline plasticizer comprises ethylene glycol dibenzoate.
8. A toner image receiving member according to claim 7 wherein said ethylene glycol dibenzoate is blended with diphenyl phthalate.
9. A toner image receiving member according to claim 1 wherein said solid crystalline plasticizer comprises dimethyl isophthalate.
10. A toner receiving member according to claim 1 wherein less than about 1.5 pounds per 1,300 square feet of said solid crystalline plasticizer is present on said external surface.

\* \* \* \* \*